# EUROPEAN PATENT SPECIFICATION

(11) **EP 4 320 306 B1**
(45) Date of publication and mention of the grant of the patent: **10.09.2025**
(21) Application number: 22717944.7
(22) Date of filing: 08.04.2022
(51) Int. Cl.: D06M 13/224, D06M 13/236, D06M 15/263, D06M 15/277, D06M 13/148, D06M 23/10

(54) **METHOD FOR CONFERRING DURABLE WATER REPELLENCE TO WOVEN OR NON-WOVEN FABRIC AND WATER REPELLENT COMPOSITION**
VERFAHREN ZUR VERLEIHUNG EINER DAUERHAFTEN WASSERABWEISENDEN WIRKUNG AUF WEB- ODER VLIESSTOFF UND WASSERABWEISENDE ZUSAMMENSETZUNG
PROCÉDÉ PERMETTANT DE CONFÉRER UNE RÉSISTANCE À L'EAU DURABLE À UN TISSU TISSÉ OU NON TISSÉ ET COMPOSITION HYDROFUGE

(30) Priority: 08.04.2021 NL 2027946
(43) Date of publication of application: 14.02.2024
(73) Proprietor: Lamoral Holding B.V., 6003 DE Weert (NL)
(72) Inventor: VERWEERDEN, Theodorus Matheus Maria, 6006RD Weert (NL); BOLLEN-BOUVRIE, Lucienne, 6162GK Geleen (NL)
(74) Representative: Wittop Koning, Tom Hugo
(86) International application number: PCT/NL2022/050198
(87) International publication number: WO 2022/216158

(56) References cited:
- WO-A1-2016/000831
- CA-A1- 3 127 531
- CN-A- 106 515 129
- CN-A- 109 023 947
- CN-A- 111 576 043

## Description

The invention relates to a method for conferring durable water repellence to woven or non-woven fabric, to a composition for conferring durable water repellence to woven or non-woven fabric and to woven or non-woven fabric treated with the said composition.

Methods for conferring durable water repellence to woven or non-woven fabric are known in the art. Up to now, the provision of durable water repellence to fabric has relied on fluorocarbon-based treatments that are highly effective and extraordinarily durable. However, the by-products such as fluor surfactants and derivatives based on C8 and C6 fluor surfactants are toxic and persist in the environment, a combination that makes it unacceptable despite its excellent performance. Many coatings that are fluor-free today have a short life span. A water repellent rain shell functionally degrades into a wind shell long before the garment itself wears out.

JP2020153057 describes a vinyl-based polymerisation of a specific divinyl compound with a molecular weight of 600 or more involving chemical bonding of the vinyl polymer to polyester fabric. An additional film is applied, comprising a fluorinated copolymer or an acrylic monomer that is polymerized with a perfluoroalkyl group having 6 or less carbon atoms. The additional film is crosslinked by a melamine resin.

EP3919673 or CA-A-3127531 describes a special fabric surface that resembles the surface of lotus flower leaves to mimic the water repellence thereof. This artificial lotus-like surface can be treated by commonly known water repellents.

WO2016/000831 describes a composition for application on textiles to confer water repellence, wherein three different acrylate monomers, one of which containing fluorine, are polymerized to a polyacrylate by the aid of an azo initiator. Apart from the thus obtained polyacrylate, the composition comprises a wax.

The present invention provides method for conferring durable water repellence to woven or non-woven fabric and a fibre treatment composition that can impart water repellence having excellent washing durability to a fibre product without the need to incorporate fluor components for water repellence, and without the need for use of silicone, isocyanates or melamine boosters. The present method for conferring durable water repellence to woven or non-woven fabric results in a highly durable and sustainable water repellent coating on the fabric, that remains unaffected even after 100 or more rounds of machine washing.

Further methods and compositions for imparting water repellence to fabrics are disclosed in CN-A-111576043 or CN-A-109023947.

To this end, the method comprises the following steps:
i) treating the fabric with an aqueous composition free of silicon compounds, the composition comprising:
   a. an aqueous solvent comprising at least 80 w/w% water, and 20 w/w% or less of a water miscible organic solvent comprising at least two functional OH groups, and
   b. 0.1 - 40 w/w% of an acrylic ester having the formula 1: wherein A¹ is H or CH₃. and A² is C₁-C₃₀ linear or branched, saturated or unsaturated hydrocarbon that may have an alicyclic or aromatic ring, the acrylic ester being dissolved, emulsified or dispersed in the aqueous solvent,
ii) heating the treated fabric to 120 - 200°C.

According to the method of the present invention, the water miscible solvent participates in a chemical reaction with the acrylic ester through the functional OH groups thereof.

By the heat treatment step ii), a (trans)esterification reaction is initiated between a water miscible solvent molecule and the acrylic ester. A covalent C-O-C bond is formed between one of the at least two OH groups of the water miscible solvent molecule and with the oxygen of the C=O group of the acrylic ester of formula 1. Since the water miscible solvent molecule has at least two functional OH groups, the acrylic ester acquires a functional OH group, enabling the said ester to bond with the fabric fibre by this OH group through hydrogen bridging. With 'functional OH group' is therefore meant that the said group is capable of forming the said C-O-C bond. The conditions are chosen such, that the above reaction or reactions can take place, e.g. at acid pH.

Without being bound to any scientific explanation, it is also possible that the transesterification reaction proceeds, wherein the aqueous solvent molecule becomes esterified with the CH₂=C(A¹)COO moiety of the acrylate ester, and the A² moiety to become covalently linked to a terminal OH group. In the latter case, the A² moiety binds to the fibric fibre by hydrogen bridging of its newly acquired terminal OH group. It is also possible that the transesterification reaction results in both, i.e. an incomplete and a complete esterification process, both resulting in the fibre acquiring a hydrophobic A² moiety bound thereto through hydrogen bridging. Since the result of the heat treatment is that the A₂ moieties become bound to the fabric, this step is also to be regarded as a curing step.

It is however clear that the composition of the present invention does not comprise an acrylate polymer, i.e. a polymer comprising a plurality of acrylate monomers, in particular three or more, polymerized to one another, e.g. by the use of an azo initiator. Further, by the above definition, it is also clear that the said acrylic ester is free of fluorine groups.

Suitable acrylic esters as defined above for step i)b. are known in the art, such as Unidyne XF series (Daikin, Japan).

The heat treatment results in a fabric, the fibres of which comprising hydrophobic A² moieties stably bound thereto through hydrogen bridging, therewith acquiring a very strong and sustainable water repellence.

The water miscible solvent can comprise more than 2 functional OH groups, but the presence of 2 functional OH groups is preferred. Accordingly, the water soluble aqueous solvent is preferably an organic water miscible solvent, more preferably chosen from the group, consisting of: ethylene glycol, ethylene glycol monomethyl ether, ethylene glycol monoethyl ether, ethylene glycol monobutyl ether, ethylene glycol monomethyl ether acetate, ethylene glycol monoethyl ether acetate, ethylene glycol monobutyl ether acetate, propylene glycol, propylene glycol monomethyl ether, propylene glycol monoethyl ether, propylene glycol dimethyl ether, dipropylene glycol, dipropylene glycol monomethyl ether, dipropylene glycol dimethyl ether, dipropylene glycol monoethyl ether, tripropylene glycol, tripropylene glycol monomethyl ether, polypropylene glycol and hexylene glycol. Most preferred is tripropylene glycol.

The aqueous solvent preferably comprises at least 0.1 w/w% of the water miscible solvent, preferably at least 0.2 w/w%.

The aqueous solvent preferably comprises 90 - 99.9 w/w% water and 0.1 - 10 w/w% of the water miscible solvent, more preferably 95 - 99.8 w/w% water and 0.2 - 5 w/w% of the water miscible solvent, or 95 - 99 w/w% water and 1 - 5 w/w% miscible organic solvent.

The composition preferably comprises 0.2 - 20 w/w% acrylic ester, more preferably 0.5 - 10 w/w%, even more preferably 1 - 6 w/w%.

For optimal water repellence, the surface tension of the coating should be about 25 mN/m². To this end, the A² moiety is preferably alkyl. The A² moiety of the acrylic ester preferably has 12 to 24 carbon atoms, more preferably 12 to 21 carbon atoms, even more preferably 18 carbon atoms. A -CH₂- moiety confers about 31 mN/m², whereas a terminal -CH₃ confers 22 mN/m². This means that a higher -CH₃ content will result in a coating with a lower surface tension and therewith to a stronger water repellence. A higher -CH₃ content can be obtained by increasing the number of branches in the hydrocarbon chain. Therefore, although the A² moiety can be linear, the said moiety is preferably branched.

It has been found that a coating applied to a fabric according to the above method remain very stably attached to the fabric. It was observed that the fabric remained fully preserved during 100 washing cycles, followed by drying in a tumble dryer operated with a regular drying program, i.e. involving heating. It was however observed that the coating started to wear after about 10 washing cycles when drying was performed without added heating (so-called "line drying").

The coating could be further improved by including a polyisocyanate having at least 3 crosslinking isocyanate groups in the aqueous composition. It was surprisingly found that the presence of polyisocyanate resulted in a significant increased stability of the coating, without any noticeable wear after 30 washing cycles followed by line drying. The functional OH groups of both the water miscible solvent molecules and of the acrylic ester comprising a functional OH group as a result of the above described transesterification reaction, as well as the A₂ moiety with a functional OH group obtained this way are covalently bound to the polyisocyanate, resulting in a crosslinked web of hydrophobic carbohydrate moieties, the web being formed by interconnection of the polyisocyanate molecules linked to one another via covalent linkage with the functional OH groups of the water miscible solvent molecules. Since these molecules comprise 2 or more functional OH groups, these function to link polyisocyanate molecules to one another, to form a hydrogen bridge bond with the fabric fibre, and to provide a functional group to the acrylic ester of the A₂ moiety, respectively.

The polyisocyanate can e.g. be aromatic or aliphatic, and suitable polyisocyanates are known in the art. Since the polyisocyanate is in an aqueous composition, e.g. water-based, the polyisocyanate is preferably blocked, e.g. by blocking groups known in the art, such as phenol, nonyl phenol, methylethylketoxime (MEKO), alcohols, ε-caprolactam, amides, imidazoles, or pyrazoles. JP2020007657 describes a fibre treatment composition containing a water repellent and such a blocked polyisocyanate. In order for the blocked polyisocyanates to become active, i.e. to become unblocked, the water is to be removed first, e.g. by drying, followed by a subsequent heating step. A very attractive isocyanate is a trimer based on aliphatic hexamethylene-1,6-diisocyanate, in particular HDI trimer (Kowa, NY, US).

The weight ratio acrylic ester : isocyanate is 100 : 5 - 100, preferably 100 : 30 - 80, more preferably 100 : 50 - 70, most preferably 100 : 60. It was found that a relatively high ratio acrylic ester : isocyanate results in the most stable coating.

In step ii), the heating is preferably performed at 130 - 200°C, more preferably 140 - 200°C, more preferably 145 - 200°C 180°C, even more preferably at 145 - 180°C, still even more preferably at 150 - 170°C and most preferably around 160°C. It has been found that such a heating step result in an excellent reaction between the components (water miscible solvent, and acrylic ester, and if present, the polyisocyanate) and binding to the fabric. In case of the presence of a blocked polyisocyanate in the composition, the said polyisocyanate becomes unblocked at such a temperature as well.

The optimal heating temperature may also depend on the treated fabric. In case of e.g. an ultra high molecular weight polyethylene, the heating temperature is preferably kept below 140°C, in particular around 130°C, since above the said temperature, deformation of the material can take place. For other fabrics that are more temperature resistant, the drying temperature is preferably higher, as described above, most preferably around 160°C. The heating step can be performed by exposure of the treated fabric to a hot air stream, or by residing in a heat chamber, or e.g. by ironing. The skilled person will be aware of the proper temperature choice. The heating step is preferably performed for 30 seconds to 10 minutes, preferably for 1 - 3 minutes.

It is preferred that the fabric as treated in step i) is dried before being subjected to the heating step ii). Such a pre-drying step becomes particularly important in the presence of a polyisocyanate, since the crosslinking reaction is preferably to be performed in a water free environment. In case there is no isocyanate present in the composition, it becomes also possible to combine the heating with the drying. However, drying can usually take place at a lower temperature than heating. Heating is preferably as described above, e.g. between 120°C and 200°C, or at 145 - 200°C, whereas drying preferably takes place preferably between 100 and 140°C, preferably below 140°C. Such a pre-drying step may therefore be more energy saving. Drying is preferably carried out for about 1 - 10 minutes, preferably about 1 - 3 minutes.

In a very attractive embodiment, the composition is also free of melamine compounds, and for the sole function of water repellence, the composition is preferably fluorine free as well. This means that there are no compounds present in the composition that have fluorine groups in their molecular backbone.

However, in order to provide a stable and wear resistant coating that is not only water repellent but also oil repellent, the composition of the invention comprises in an attractive embodiment a fluorinated C₂-C₂₀ alkyl compound comprising a terminal acryl group, as e.g. is described in JP2020153057, and as are known in the art, e.g. The Unidyne TG Series (Daikin, Japan). By including such a fluor acrylic ester in the composition, this fluor acrylic ester will be susceptible to the transesterification reaction with the water miscible solvent as the fluorine free acrylic ester of formula 1 as described above, and will therefore result in a fluorinated hydrocarbon moiety bound to the fabric fibre through hydrogen bridging, and be able to participate in the crosslinking with the polyisocyanate, if present.

By the provision of such a fluorinated acrylic ester, not only water repellence, but also oil repellence is obtained. Very attractively, the fluorinated alkyl compound is defined as the fluorine free acrylic ester of formula 1, wherein for the fluorinated compound, the A2 moiety is a C₆-C₂₀ alkyl, 1 to 6 of the carbon atoms being fully substituted with fluorine. The term 'fully substituted with fluorine' means that all the H atoms of the respective carbon atom have been replaced by a fluorine atom. A saturated terminal carbon atom will, when fully substituted, have three fluorine atoms, and a saturated internal carbon, i.e. flanked by two adjacent carbon atoms by a single bond, will have two fluorine atoms. This means that the fluorine groups can be scattered throughout the alkyl backbone. Such compounds are e.g. known from WO2016/096128. Very attractively, the A₂ of the fluorinated compound is a C₆ alkyl, all 6 of the carbon atoms being fully substituted with fluorine.

Since the surface tension of -CF₂- groups is 18 mN/m², and of terminal -CF₂ and -CF₃ groups is 15 mN/m² and 6 mN/m², respectively, a branched fluorinated alkyl compound with terminal -CF₂ and -CF₃ groups, in particular -CF₃ groups is preferred.

The composition preferably comprises in w/w% an equal amount of both non-fluorinated and fluorinated acrylic esters. The composition preferably comprises 0.2 - 20 w/w% acrylic ester, more preferably 0.5 - 10 w/w%, even more preferably 1 - 6 w/w% of the fluorinated C₂-C₂₀ alkyl compound. In case of the presence of a fluorinated acrylic ester, the weight ratio of isocyanate, if present, to acrylic acid is determined by the sum of both the fluorinated and fluor free acrylic esters present in the composition.

The method of the invention can also be applied to fabric fibres before being assembled to a fabric or textile, instead of treatment of the fabric or textile. A similar water repellence is obtained when a fabric or textile is produced from such treated fibres.

The fibres and/or the fabric is preferably chosen from polyester, polyamide, acrylate, ultra high molecular weight polyethylene (e.g. Dyneema, DSM, Netherlands), cotton or aramide or a mixture of two or more thereof. It was found that the repellent coating was stably and strongly bonded to these types of fabric. To this end, the fabric preferably comprises polyester and/or polyamide, more preferably polyester.

The treatment of step i) is preferably chosen from dipping the fabric in the composition, or spraying the composition onto the fabric. Dipping means that the fabric is immersed in the composition. Dipping is preferred, but spraying is a very attractive home appliance, where the fabric can be sprayed from an aerosol comprising the composition, whereafter the heat treatment can be performed by ironing. In an industrial setting, the treated fabric is preferably dipped and padded subsequently, in order to remove superfluous liquid composition.

In another aspect, the invention relates to a composition free of fluorine and silicone as defined in the appended claims for conferring durable water repellence to woven or non-woven fabrics.

In still another aspect, the invention relates to fibres, woven or non-woven fabric as described herein, treated with the composition as defined in the appended claims.

The invention will now be further illustrated by way of examples and figure, showing a possible industrial set up for the method of the invention.

The arrows reflect the transportation direction of the fabric 1, guided by guidance rollers 2. The process is continuous, e.g. without interruption. Fabric 1 is immersed in a bath 3 comprising the composition 4 of the invention. After leaving the bath 3, the fabric 4 passes through two padding rolls 5, squeezing the superfluous liquid composition from the fabric. The fabric is dried with hot air in drying chamber 6, where the temperature is e.g. 130°C, and eventually enter a heating chamber, where the temperature is e.g. 160°C.

### Examples

### Water repellence

Samples of PES 1 fabric 135 gr/m² and PES 2 fabric 190 gr/m² (MB Sportswear, Eindhoven Netherlands) were washed 100 times according to the method of Iso 6330 3G or 4H.

After washing, the water repellence is measured by the ISO 4920 (version 2012-12) spray method

### Commercial washing cycles:

The water repellence measured by the Iso 4920 spray method after washing 120 times according to the method of using a commercial washing machine of the type Miele Twindos (Germany) using the program Express 2.0 and the detergent Colour Reus extra strong against stains, extra clean (Henkel, Germany). The program specifications and the contents of the detergent are given in tables 1 and 2, respectively.

**Table 1: Washing program**

| | |
|---|---|
| washing time | 6 min. |
| rinsing time | 14 min. |
| pumping time | 14 min. |
| spinning time | 1 min. |
| washing cycle time | 27 min. |
| load | 2 - 3 kg |
| temperature | 30°C |

**Table 2: Ingredients detergent**

| |
|---|
| anionic surface active agents (5-15%) |
| soap (< 5 %) |
| non ionic surface active agents |
| phoshonates |
| parfumes |
| hexl cynnamal |
| conservation agents |
| methylisothiazolinone |
| benzisothiazolinone |
| enzymes |

### Oil repellence

Oil repellence is measure after washing 100 times of samples as described above according to the AATCC118 method 118-1997.

### Sample preparation

The fabric sample was cut 15 x 15 cm from the reel and by dipping the fabric for 1 minute in the coating emulsion. The uncoated fabric was weighed *in duplo.* After dipping, the coated sample was placed on a rubber sleeve of a manual coating unit (RK prints) for the padding process. With a smooth roller with a weight of 10 kg the excess of emulsion was squeezed out by 2 times rolling the roller over the fabric.

The samples were dried in an oven with forced air ventilation for 3 minutes at 130°C ; subsequently the sample was cured for 1 minute at 160°C. After curing, the sample was weighted *in duplo* again.

Possible compositions for use in examples 1 - 8 are given in table 3. The experiment have been performed with the compositions given in table 4.

In examples 1, 3, 5 - 10, a polyester woven fabric PES 135 gr/m² ('pique') (MB Sportswear, Eindhoven Netherlands) was used, whereas in examples 2 and 4 195 gr/m² 'smooth' (MB Sportswear, Eindhoven Netherlands) was used.

It was observed that all examples, after the washing cycles and drying in a tumble dryer (AEG Lavatherm Protex plus, AEG, Germany, with the program setting 'cotton extra dry') retained their water repellence. Grade iso 5 was measured for all samples before the first washing and after 100 or 120 times washing. Grade 5 means that no sticking or wetting of the upper surface was observed.

The same was true for examples 1 and 3 when the dipping was replaced by spraying and the padding was replaced by tumbling in a tumble dryer as described above. Heating was performed by ironing at 150°C (level**) for example 1 and at 200°C (level***) for example 2, in conformity with the ironing prescriptions of the fabric manufacturer. Also for these samples, Grade iso 5 was measured for all samples before the first washing and after 100 or 120 times washing.

The oil repellence for examples 3, 4, 8 - 10 as measured according to AATCC118 was grade 5 - 6 after 100 - 120 times washing followed by the above tumble drying.

It was however observed that in case of line drying, i.e. without heating the dried fabric, a coating that has been subjected to crosslinking with polyisocyanate remained stably bound as compared to the results for all coatings after tumble drying, whereas the coatings without comprising the isocyanate (NCO) crosslinkages tended to loosen from the fabric after 10 - 12 washing cycles, see table 5. It was observed that a weight ratio acrylic ester : polyisocyanate of above 30 gave the best bonding.

**Table 5**

| | 0 | 3 | 6 | 9 | 12 | 15 | 18 | 21 | 24 | 27 | 30 |
|---|---|---|---|---|---|---|---|---|---|---|---|
| Example 1 (no NCO) | 5 | 5 | 5 | 5 | 4 | 3 | 3 | 3 | 2 | 2 | 2 |
| Example 5 (100 : 60) | 5 | 5 | 5 | 5 | 5 | 5 | 5 | 5 | 5 | 5 | 5 |
| Example 6 (100 : 30) | 5 | 5 | 5 | 5 | 5 | 4,5 | 3 | 3 | 3 | 2 | 3 |
| Example 7 (100 : 10) | 5 | 5 | 5 | 5 | 5 | 4 | 4,5 | 4 | 3 | 3 | 2 |

## Claims

1. Method for conferring durable water repellence to woven or non-woven fabric, comprising the steps of:
- treating the fabric with an aqueous composition free of silicon compounds, the composition comprising:
a. an aqueous solvent comprising at least 80 w/w% water, and 20 w/w% or less of a water miscible organic solvent comprising at least two functional OH groups, and
b. 0.1 - 40 w/w% of an acrylic ester having the formula 1: wherein A¹ is H or CH₃, and A² is C₁-C₃₀ linear or branched, saturated or unsaturated hydrocarbon that may have an alicyclic or aromatic ring, the acrylic ester being dissolved, emulsified or dispersed in the aqueous solvent,
- heating the treated fabric to 120 - 200°C.

2. Method of claim 1, wherein
- the water miscible solvent is chosen from the group, consisting of: ethylene glycol, ethylene glycol monomethyl ether, ethylene glycol monoethyl ether, ethylene glycol monobutyl ether, ethylene glycol monomethyl ether acetate, ethylene glycol monoethyl ether acetate, ethylene glycol monobutyl ether acetate, propylene glycol, propylene glycol monomethyl ether, propylene glycol monoethyl ether, propylene glycol dimethyl ether, dipropylene glycol, dipropylene glycol monomethyl ether, dipropylene glycol dimethyl ether, dipropylene glycol monoethyl ether, tripropylene glycol, tripropylene glycol monomethyl ether, polypropylene glycol and hexylene glycol, the water miscible solvent preferably comprising tripropylene glycol; and/or
- the aqueous solvent comprises 90 - 99.9 w/w% water and 0.1 - 10 w/w% of the water miscible solvent, preferably 95 - 99.8 w/w% water and 0.2 - 5 w/w% of the water miscible solvent, or 95 - 99 w/w% water and 1 - 5 w/w% miscible organic solvent.

3. Method of claim 1 or 2, wherein
- the composition comprises 0.2 - 20 w/w% acrylic ester, preferably 0.5 - 10 w/w%, more preferably 1 - 6 w/w%; and/or
- A² of the acrylic ester has 12 to 24 carbon atoms, preferably 12 to 21 carbon atoms, more preferably 18 carbon atoms; and/or
- A² of the acrylic ester is alkyl; and/or
- A² of the acrylic ester is branched.

4. Method of any of the preceding claims, further comprising a polyisocyanate comprising at least 3 crosslinkable isocyanate groups,
- the polyisocyanate preferably being a water-based blocked polyisocyanate; and/or
- the weight ratio acrylic ester : isocyanate preferably being 100 : 5 - 100, more preferably 100 : 30 - 80, even more preferably 100 : 50 - 70, and most preferably 100 : 60.

5. Method of any of the preceding claims, wherein
- the treated fabric of step i) is dried before step ii), and/or
- the fabric preferably being dried at 100 - 140°C; and/or
- in step ii) the heating preferably being performed at 130 - 200°C, more preferably 140 - 200°C, more preferably at 145 - 200°C, even more preferably at 145 - 180°C, still more preferably at 150 - 170°C; and/or
- the heating step preferably being performed for 30 seconds to 10 minutes.

6. Method of any of the preceding claims, wherein the composition is free of melamine compounds and/or is fluorine free.

7. Method of any of the claims 1 - 5, wherein the composition further comprises a fluorinated C₂-C₂₀ alkyl compound comprising a terminal acryl group;
- the fluorinated alkyl compound preferably being a C₆-C₂₀ alkyl, 1 to 6 of the carbon atoms being fully substituted with fluorine; and/or
- the fluorinated alkyl compound preferably being branched; and/or
- the composition preferably comprising in w/w% an equal amount of both non-fluorinated and fluorinated acrylic esters.

8. Method of any of the preceding claims, wherein the fabric is chosen from polyester, polyamide, acrylate, ultra high molecular weight polyethylene, cotton or aramide or a mixture of two or more thereof, the fabric preferably comprising polyester and/or polyamide, more preferably polyester.

9. Method of any of the preceding claims, wherein
- the treatment of step i) is chosen from dipping the fabric in the composition, or spraying the composition onto the fabric; and/or
- the treated fabric is padded before being dried or heated.

10. Composition free of fluorine and silicon compounds for conferring durable water repellence to woven or non-woven fabric, the composition comprising
a. an aqueous solvent comprising at least 80 w/w% water, and 20 w/w% or less of a water miscible organic solvent comprising at least two functional OH groups, and
b. 0.1 - 40 w/w% of an acrylic ester having the formula 1: wherein A¹ is H or CH₃, and A² is C₁-C₃₀ linear or branched, saturated or unsaturated hydrocarbon that may have an alicyclic or aromatic ring, the acrylic ester being dissolved, emulsified or dispersed in the aqueous solvent.

11. Composition of claim 10, wherein
- the water miscible solvent is chosen from the group, consisting of: ethylene glycol, ethylene glycol monomethyl ether, ethylene glycol monoethyl ether, ethylene glycol monobutyl ether, ethylene glycol monomethyl ether acetate, ethylene glycol monoethyl ether acetate, ethylene glycol monobutyl ether acetate, propylene glycol, propylene glycol monomethyl ether, propylene glycol monoethyl ether, propylene glycol dimethyl ether, dipropylene glycol, dipropylene glycol monomethyl ether, dipropylene glycol dimethyl ether, dipropylene glycol monoethyl ether, tripropylene glycol, tripropylene glycol monomethyl ether, polypropylene glycol and hexylene glycol, the water miscible solvent preferably comprising tripropylene glycol;
- the aqueous solvent comprises 90 - 99.9 w/w% water and 0.1 - 10 w/w% of the water miscible solvent, preferably 95 - 99.8 w/w% water and 0.2 - 5 w/w% of the water miscible solvent, or 95 - 99 w/w% water and 1 - 5 w/w% miscible organic solvent.

12. Composition of any of the claims 10 or 11, wherein
- the composition comprises 0.2 - 20 w/w% acrylic ester, preferably 0.5 - 10 w/w%, more preferably 1 - 6 w/w%; and/or
- A² of the acrylic ester has 12 to 24 carbon atoms, preferably 12 to 21 carbon atoms, more preferably 18 carbon atoms; and/or
- A² of the acrylic ester is alkyl; and/or
- A² of the acrylic ester is branched.

13. Composition of any of the claims 10 - 12, further comprising a polyisocyanate comprising at least 3 crosslinkable isocyanate groups,
- the polyisocyanate preferably being a water-based blocked polyisocyanate; and/or
- the weight ratio acrylic ester : isocyanate preferably being 100 : 5 - 100, more preferably 100 : 30 - 80, even more preferably 100 : 50 - 70, and most preferably 100 : 60.

14. Composition of any of the claims 10 - 13, wherein the composition is free of silicon and melamine compounds.

15. Woven or non-woven fabric, treated with the composition of any of the claims 10 - 14, the fabric preferably being chosen from polyester, polyamide, acrylate, ultra high molecular weight polyethylene, cotton or aramide or a mixture of two or more thereof, the fabric preferably comprising polyester and/or polyamide, more preferably polyester.

## Patentansprüche

1. Verfahren zum Verleihen einer dauerhaften Wasserabweisung an gewebte oder nicht gewebte Stoffe, umfassend die folgenden Schritte:
- Behandeln des Stoffes mit einer wässrigen Zusammensetzung, die frei von Siliciumverbindungen ist, wobei die Zusammensetzung umfasst:
a. ein wässriges Lösungsmittel, das mindestens 80 Gew.-% Wasser und 20 Gew.-% oder weniger eines mit Wasser mischbaren organischen Lösungsmittels umfasst, das mindestens zwei funktionelle OH-Gruppen umfasst, und
b. 0,1 bis 40 Gew.-% eines Acrylesters der Formel 1: worin A¹ H oder CH₃ ist und A² ein linearer oder verzweigter, gesättigter oder ungesättigter C₁-C₃₀-Kohlenwasserstoffrest ist, der einen alicyclischen oder aromatischen Ring aufweisen kann, wobei der Acrylester in dem wässrigen Lösungsmittel gelöst, emulgiert oder dispergiert ist,
- Erhitzen des behandelten Gewebes auf 120 bis 200°C.

2. Verfahren nach Anspruch 1, wobei
- das wassermischbare Lösungsmittel ausgewählt ist aus der Gruppe bestehend aus: Ethylenglykol, Ethylenglykolmonomethylether, Ethylenglykolmonoethylether, Ethylenglykolmonobutylether, Ethylenglykolmonomethyletheracetat, Ethylenglykolmonoethyletheracetat, Ethylenglykolmonobutyletheracetat, Propylenglykol, Propylenglykolmonomethylether, Propylenglykolmonoethylether, Propylenglykoldimethylether, Dipropylenglykol, Dipropylenglykolmonomethylether, Dipropylenglykoldimethylether, Dipropylenglykolmonoethylether, Tripropylenglykol, Tripropylenglykolmonomethylether, Polypropylenglykol und Hexylenglykol, wobei das wassermischbare Lösungsmittel vorzugsweise Tripropylenglykol umfasst; und/oder
- das wässrige Lösungsmittel 90 - 99,9 Gew.-% Wasser und 0,1 - 10 Gew.-% des wassermischbaren Lösungsmittels, vorzugsweise 95 - 99,8 Gew.-% Wasser und 0,2 - 5 Gew.-% des wassermischbaren Lösungsmittels oder 95 - 99 Gew.-% Wasser und 1 - 5 Gew.-% mischbares organisches Lösungsmittel umfasst.

3. Verfahren nach Anspruch 1 oder 2, wobei
- die Zusammensetzung 0,2 bis 20 Gew.-% Acrylester, vorzugsweise 0,5 bis 10 Gew.-%, noch bevorzugter 1 bis 6 Gew.-%, umfasst; und/oder
- A² des Acrylesters 12 bis 24 Kohlenstoffatome, vorzugsweise 12 bis 21 Kohlenstoffatome, noch bevorzugter 18 Kohlenstoffatome aufweist; und/oder
- A² des Acrylesters Alkyl ist; und/oder
- A² des Acrylesters verzweigt ist.

4. Verfahren nach einem der vorstehenden Ansprüche, das ferner ein Polyisocyanat umfasst, das mindestens 3 vernetzbare Isocyanatgruppen umfasst, wobei
- das Polyisocyanat vorzugsweise ein wasserbasiertes blockiertes Polyisocyanat ist; und/oder
- das Gewichtsverhältnis Acrylester : Isocyanat vorzugsweise 100 : 5 - 100, noch bevorzugter 100 : 30 - 80, noch mehr bevorzugt 100 : 50 - 70 und am meisten bevorzugt 100 : 60 beträgt.

5. Verfahren nach einem der vorstehenden Ansprüche, wobei
- das behandelte Gewebe aus Schritt i) vor Schritt ii) getrocknet wird, und/oder
- das Gewebe vorzugsweise bei 100-140°C getrocknet wird; und/oder
- in Schritt ii) die Erwärmung vorzugsweise bei 130 - 200°C, noch bevorzugter bei 140 - 200°C, noch bevorzugter bei 145 - 200°C, noch bevorzugter bei 145 - 180°C, noch bevorzugter bei 150 - 170°C durchgeführt wird; und/oder
- wobei der Erhitzungsschritt vorzugsweise 30 Sekunden bis 10 Minuten lang durchgeführt wird.

6. Verfahren nach einem der vorstehenden Ansprüche, wobei die Zusammensetzung frei von Melaminverbindungen und/oder fluorfrei ist.

7. Verfahren nach einem der Ansprüche 1 bis 5, wobei die Zusammensetzung ferner eine fluorierte C₂-C₂₀-Alkylverbindung mit einer endständigen Acrylgruppe umfasst;
- wobei die fluorierte Alkylverbindung vorzugsweise eine C₆-C₂₀-Alkylverbindung ist, wobei 1 bis 6 der Kohlenstoffatome vollständig durch Fluor substituiert sind; und/oder
- wobei die fluorierte Alkylverbindung vorzugsweise verzweigt ist; und/oder
- wobei die Zusammensetzung vorzugsweise in Gew.-% eine gleiche Menge an nicht fluorierten und fluorierten Acrylestern umfasst.

8. Verfahren nach einem der vorstehenden Ansprüche, wobei das Gewebe ausgewählt ist aus Polyester, Polyamid, Acrylat, ultrahochmolekularem Polyethylen, Baumwolle oder Aramid oder einer Mischung aus zwei oder mehr davon, wobei das Gewebe vorzugsweise Polyester und/oder Polyamid, noch bevorzugter Polyester umfasst.

9. Verfahren nach einem der vorstehenden Ansprüche, wobei
- die Behandlung in Schritt i) ausgewählt ist aus dem Eintauchen des Gewebes in die Zusammensetzung oder dem Aufsprühen der Zusammensetzung auf das Gewebe; und/oder
- das behandelte Gewebe vor dem Trocknen oder Erhitzen gepolstert wird.

10. Zusammensetzung, die frei von Fluor- und Siliciumverbindungen ist, zum Verleihen einer dauerhaften Wasserabweisung an gewebte oder nicht gewebte Stoffe, wobei die Zusammensetzung umfasst
a. ein wässriges Lösungsmittel, das mindestens 80 Gew.-% Wasser und 20 Gew.-% oder weniger eines mit Wasser mischbaren organischen Lösungsmittels umfasst, das mindestens zwei funktionelle OH-Gruppen umfasst, und
b. 0,1 bis 40 Gew.-% eines Acrylesters der Formel 1: worin A¹ H oder CH₃ ist und A² ein linearer oder verzweigter, gesättigter oder ungesättigter C₁-C₃₀-Kohlenwasserstoff ist, der einen alicyclischen oder aromatischen Ring aufweisen kann, wobei der Acrylester in dem wässrigen Lösungsmittel gelöst, emulgiert oder dispergiert ist.

11. Zusammensetzung nach Anspruch 10, wobei
- das wassermischbare Lösungsmittel ausgewählt ist aus der Gruppe bestehend aus: Ethylenglykol, Ethylenglykolmonomethylether, Ethylenglykolmonoethylether, Ethylenglykolmonobutylether, Ethylenglykolmonomethyletheracetat, Ethylenglykolmonoethyletheracetat, Ethylenglykolmonobutyletheracetat, Propylenglykol, Propylenglykolmonomethylether, Propylenglykolmonoethylether, Propylenglykoldimethylether, Dipropylenglykol, Dipropylenglykolmonomethylether, Dipropylenglykoldimethylether, Dipropylenglykolmonoethylether, Tripropylenglykol, Tripropylenglykolmonomethylether, Polypropylenglykol und Hexylenglykol, wobei das wassermischbare Lösungsmittel vorzugsweise Tripropylenglykol umfasst;
- das wässrige Lösungsmittel 90 - 99,9 Gew.-% Wasser und 0,1 - 10 Gew.-% des wassermischbaren Lösungsmittels, vorzugsweise 95 - 99,8 Gew.-% Wasser und 0,2 - 5 Gew.-% des wassermischbaren Lösungsmittels oder 95 - 99 Gew.-% Wasser und 1 - 5 Gew.-% mischbares organisches Lösungsmittel umfasst.

12. Zusammensetzung nach einem der Ansprüche 10 oder 11, wobei
- die Zusammensetzung 0,2 bis 20 Gew.-% Acrylester, vorzugsweise 0,5 bis 10 Gew.-%, noch bevorzugter 1 bis 6 Gew.-%, umfasst; und/oder
- A² des Acrylesters 12 bis 24 Kohlenstoffatome, vorzugsweise 12 bis 21 Kohlenstoffatome, noch bevorzugter 18 Kohlenstoffatome aufweist; und/oder
- A² des Acrylesters Alkyl ist; und/oder
- A² des Acrylesters verzweigt ist.

13. Zusammensetzung nach einem der Ansprüche 10 bis 12, die zusätzlich ein Polyisocyanat umfasst, das mindestens 3 vernetzbare Isocyanatgruppen umfasst, wobei
- das Polyisocyanat vorzugsweise ein wasserbasiertes blockiertes Polyisocyanat ist; und/oder
- wobei das Gewichtsverhältnis Acrylester : Isocyanat vorzugsweise 100 : 5 - 100, noch bevorzugter 100 : 30 - 80, noch mehr bevorzugt 100 : 50 - 70 und am meisten bevorzugt 100 : 60 beträgt.

14. Zusammensetzung nach einem der Ansprüche 10 bis 13, wobei die Zusammensetzung frei von Silizium- und Melaminverbindungen ist.

15. Gewebter oder nicht gewebter Stoff, der mit der Zusammensetzung nach einem der Ansprüche 10 bis 14 behandelt ist, wobei der Stoff vorzugsweise aus Polyester, Polyamid, Acrylat, ultrahochmolekularem Polyethylen, Baumwolle oder Aramid oder einer Mischung aus zwei oder mehr davon ausgewählt ist, wobei der Stoff vorzugsweise Polyester und/oder Polyamid, noch bevorzugter Polyester umfasst

## Revendications

1. Procédé pour conférer une hydrofugation durable à un tissu tissé ou non-tissé, comprenant les étapes suivantes :
- traiter le tissu avec une composition aqueuse exempte de composés de silicium, la composition comprenant :
a. un solvant aqueux comprenant au moins 80 % en poids d'eau et 20 % en poids ou moins d'un solvant organique miscible à l'eau comprenant au moins deux groupes fonctionnels OH, et
b. 0,1 à 40 % en poids d'un ester acrylique répondant à la formule 1 : dans laquelle A¹ représente H ou CH₃, et A² représente un groupe hydrocarboné linéaire ou ramifié, saturé ou insaturé en C₁ à C₃₀ pouvant comporter un cycle alicyclique ou aromatique, l'ester acrylique étant dissous, émulsionné ou dispersé dans le solvant aqueux,
- chauffage du tissu traité à une température comprise entre 120 et 200 °C.

2. Procédé selon la revendication 1, dans lequel
- le solvant miscible à l'eau est choisi dans le groupe constitué par : l'éthylène glycol, l'éthylène glycol monométhyl éther, l'éthylène glycol monoéthyl éther, l'éthylène glycol monobutyl éther, l'acétate d'éthylène glycol monométhyl éther, l'acétate d'éthylène glycol monoéthyl éther, l'acétate d'éthylène glycol monobutyl éther, le propylène glycol, le propylène glycol monométhyl éther, propylène glycol monoéthyl éther, propylène glycol diméthyl éther, dipropylène glycol, dipropylène glycol monométhyl éther, dipropylène glycol diméthyl éther, dipropylène glycol monoéthyl éther, tripropylène glycol, tripropylène glycol monométhyl éther, polypropylène glycol et hexylène glycol, le solvant miscible à l'eau comprenant de préférence du tripropylène glycol ; et/ou
- le solvant aqueux comprend 90 à 99,9 % en poids d'eau et 0,1 à 10 % en poids du solvant miscible dans l'eau, de préférence 95 à 99,8 % en poids d'eau et 0,2 à 5 % en poids du solvant miscible dans l'eau, ou 95 à 99 % en poids d'eau et 1 à 5 % en poids de solvant organique miscible.

3. Procédé selon la revendication 1 ou 2, dans lequel
- la composition comprend 0,2 à 20 % en poids d'ester acrylique, de préférence 0,5 à 10 % en poids, plus préférablement 1 à 6 % en poids ; et/ou
- A² de l'ester acrylique a 12 à 24 atomes de carbone, de préférence 12 à 21 atomes de carbone, plus préférablement 18 atomes de carbone ; et/ou
- A² de l'ester acrylique est un groupe alkyle ; et/ou
- A² de l'ester acrylique est ramifié.

4. Procédé selon l'une quelconque des revendications précédentes, comprenant en outre un polyisocyanate comprenant au moins 3 groupes isocyanate réticulables,
- le polyisocyanate étant de préférence un polyisocyanate bloqué à base d'eau ; et/ou
- le rapport pondéral ester acrylique : isocyanate étant de préférence de 100 : 5 à 100, de préférence de 100 : 30 à 80, encore de préférence de 100 : 50 à 70, et de préférence de 100 : 60.

5. Procédé selon l'une quelconque des revendications précédentes, dans lequel
- le tissu traité de l'étape i) est séché avant l'étape ii), et/ou
- le tissu est de préférence séché à 100 - 140 °C ; et/ou
- dans l'étape ii), le chauffage est de préférence effectué à 130 - 200 °C, plus préférablement à 140 - 200 °C, plus préférablement à 145 - 200 °C, encore plus préférablement à 145 - 180 °C, encore plus préférablement à 150 - 170 °C ; et/ou
- l'étape de chauffage étant de préférence réalisée pendant 30 secondes à 10 minutes.

6. Procédé selon l'une quelconque des revendications précédentes, dans lequel la composition est exempte de composés de mélamine et/ou est exempte de fluor.

7. Procédé selon l'une quelconque des revendications 1 à 5, dans lequel la composition comprend en outre un composé alkyle fluoré en C₂ à C₂₀ comprenant un groupe acrylique terminal ;
- le composé alkyle fluoré étant de préférence un alkyle en C₆ à C₂₀, 1 à 6 des atomes de carbone étant entièrement substitués par du fluor ; et/ou
- le composé alkyle fluoré étant de préférence ramifié ; et/ou
- la composition comprenant de préférence, en % en poids, une quantité égale d'esters acryliques non fluorés et fluorés.

8. Procédé selon l'une quelconque des revendications précédentes, dans lequel le tissu est choisi parmi le polyester, le polyamide, l'acrylate, le polyéthylène à poids moléculaire ultra élevé, le coton ou l'aramide ou un mélange de deux ou plusieurs de ceux-ci, le tissu comprenant de préférence du polyester et/ou du polyamide, de préférence du polyester.

9. Procédé selon l'une quelconque des revendications précédentes, dans lequel
- le traitement de l'étape i) est choisi parmi le trempage du tissu dans la composition ou la pulvérisation de la composition sur le tissu ; et/ou
- le tissu traité est rembourré avant d'être séché ou chauffé.

10. Composition exempte de composés fluoré et de silicium pour conférer une hydrophobie durable à un tissu ou un non-tissé, la composition comprenant
a. un solvant aqueux comprenant au moins 80 % en poids d'eau et 20 % en poids ou moins d'un solvant organique miscible à l'eau comprenant au moins deux groupes fonctionnels OH, et
b. 0,1 à 40 % en poids d'un ester acrylique ayant la formule 1 : dans laquelle A¹ est H ou CH₃, et A² est un hydrocarbure en C₁ à C₃₀ linéaire ou ramifié, saturé ou insaturé, qui peut avoir un cycle alicyclique ou aromatique, l'ester acrylique étant dissous, émulsionné ou dispersé dans le solvant aqueux.

11. Composition selon la revendication 10, dans laquelle
- le solvant miscible à l'eau est choisi dans le groupe constitué par : l'éthylène glycol, l'éthylène glycol monométhyl éther, l'éthylène glycol monoéthyl éther, l'éthylène glycol monobutyl éther, l'acétate d'éthylène glycol monométhyl éther, l'acétate d'éthylène glycol monoéthyl éther, l'acétate d'éthylène glycol monobutyl éther, le propylène glycol, propylène glycol monométhyl éther, propylène glycol monoéthyl éther, propylène glycol diméthyl éther, dipropylène glycol, dipropylène glycol monométhyl éther, dipropylène glycol diméthyl éther, dipropylène glycol monoéthyl éther, tripropylène glycol, tripropylène glycol monométhyl éther, polypropylène glycol et hexylène glycol, le solvant miscible à l'eau comprenant de préférence du tripropylène glycol ;
- le solvant aqueux comprend 90 à 99,9 % en poids d'eau et 0,1 à 10 % en poids du solvant miscible dans l'eau, de préférence 95 à 99,8 % en poids d'eau et de 0,2 à 5 % en poids du solvant miscible dans l'eau, ou 95 à 99 % en poids d'eau et de 1 à 5 % en poids de solvant organique miscible.

12. Composition selon l'une quelconque des revendications 10 ou 11, dans laquelle
- la composition comprend 0,2 à 20 % en poids d'ester acrylique, de préférence 0,5 à 10 % en poids, plus préférablement 1 à 6 % en poids ; et/ou
- A² de l'ester acrylique a 12 à 24 atomes de carbone, de préférence 12 à 21 atomes de carbone, plus préférablement 18 atomes de carbone ; et/ou
- A² de l'ester acrylique est un groupe alkyle ; et/ou
- A² de l'ester acrylique est ramifié.

13. Composition selon l'une quelconque des revendications 10 à 12, comprenant en outre un polyisocyanate comprenant au moins 3 groupes isocyanate réticulables,
- le polyisocyanate étant de préférence un polyisocyanate bloqué à base d'eau ; et/ou
- le rapport pondéral ester acrylique : isocyanate étant de préférence de 100 : 5 à 100, plus préférablement de 100 : 30 à 80, encore plus préférablement de 100 : 50 à 70, et le plus préférablement de 100 : 60.

14. Composition selon l'une quelconque des revendications 10 à 13, dans laquelle la composition est exempte de silicium et de composés de mélamine.

15. Tissu tissé ou non tissé, traité avec la composition selon l'une quelconque des revendications 10 à 14, le tissu étant de préférence choisi parmi le polyester, le polyamide, l'acrylate, le polyéthylène à poids moléculaire ultra élevé, le coton ou l'aramide ou un mélange de deux ou plusieurs de ceux-ci, le tissu comprenant de préférence du polyester et/ou du polyamide, plus préférablement du polyester.
